

## UNITED STATES PATENT OFFICE

CLEO H. KIDWELL, OF DONGAN HILLS, NEW YORK, ASSIGNEE TO KIDWELL & COMPANY, INC., A CORPORATION OF NEW YORK

## PROCESS AND SOLUTION FOR THE TREATMENT OF SILK

No Drawing.

Application filed February 26 1930. Serial No. 432,367.

This invention relates to a process for the treatment of silk generally, and also for the treatment of knitted silk articles such as hosiery, sweaters and the like. It applies also to cotton and other textile materials and to articles made therefrom.

While I consider my invention to be broadly new and while it has application either to silk or other textile material in the raw state, that is, in skeins or hanks before it has been made into the finished article, or to the article itself either after or during the course of manufacture, I shall devote myself particularly in this specification to a description of the process and the improvements derived from its use when applied to women's silk hosiery. Persons skilled in the art will readily be able to apply my invention to other articles or to silk, cotton, or other textile material in its natural or raw state before it has been made up into articles.

There are a number of serious problems in the silk hosiery industry. Many attempts have been made to solve them but so far as I am aware no successful means has as yet been devised. One of the difficulties is that commonly known as picking. Picking is the pulling out or tearing loose of threads in the stocking. This results from handling the stockings and passing the fingers over their surface. When stockings are sold over the counter and handled by customers, a considerable number of them are rendered imperfect as a result of picking. The tiny loose strands of silk on the surface of the stocking make an almost imperceptible fuzz, and when the hand of the customer is passed over it certain of these strands are frequently caught and pulled loose. As a result the appearance of the stocking is injured and there is a great tendency for a run to start at this point. My invention contemplates the prevention of this difficulty to a large degree.

Another common evil in the silk hosiery industry is that known to the trade as sleazy knitting. Sleazy knitting is believed to result from an inequality of tension on the silk threads at different portions of the stocking. It is particularly common in stockings which have been knitted directly from the gummed

silk. The smooth uniform appearance so desirable in silk stockings is seriously impaired by sleazy knitting. According to my invention I treat stockings which are imperfect by reason of sleazy knitting and remove the undesirable surface appearance which it produces.

At the present time there is a great vogue for sheer stockings. The process of my invention renders stockings more sheer and thus assists towards the end which the hosiery manufacturers are seeking without necessitating the use of different machines or finer grade silk. Also, I have found that stockings which have been subjected to the process of my invention take the dye more uniformly than untreated stockings. If, therefore, my process is used before the stockings are dyed, this additional advantage can be made use of.

In practicing my invention, the silk may be treated in the gum or after the gum has been boiled off, but in either case the stocking must be dry before treating. The requirements of different manufacturers will vary as to the time which it is desired to subject the stocking to my solution. Accordingly there will be a variation in the ingredients of the solution and of the amounts thereof, depending on the time of treatment. I have found that a one-minute treatment is about right for most manufacturers, and the solution which I use in this case for Japanese mulberry silk is as follows:

99 % by volume of 85% commercial formic acid  
1 % by volume of 95% sulphuric acid  
2% (of the above volume) U. S. P. glycerine

I take the stockings in a dry condition and immerse them in the above solution for about one minute as aforesaid. I then remove the stockings and give them a thorough washing in an ammonia bath of from three to five percent by weight concentration, or other suitable alkaline solution such as milk of lime (calcium hydroxide). The duration of the bath may vary from about fifteen minutes to an hour. I have found that about one-

quarter of an hour is very satisfactory. If it is desired to preserve the strength of the alkaline solution so that it may be used for a succession of such washings, the silk should be immersed in running water for two or three minutes, or agitated in two or three still baths of water before it is transferred to the alkaline bath. A good deal of the acid is thus washed out before the alkaline bath is given.

10 After this treatment the stockings are thoroughly washed in water after which they may be dried or, if the treatment is applied in the course of manufacture, they may be sent in a wet condition to the next step in the manufacturing process. If the stockings are treated in the gum, they may be sent while still wet to the vats where the gum will be boiled off, after which they will be dyed.

15 20 It will be understood that the percentage given above and the specified strengths of the ingredients are not fixed but may be varied somewhat under different conditions of treatment and for different kinds and grades of

25 silk. For example, if it is desired to treat the stockings only a very short time, say fifteen seconds or less, it is not necessary to use glycerine or other protective agents in the solution. But when treatments of a 30 greater length of time are desired, glycerine or some other alcohol such as ethyl alcohol or other suitable protective agent should be used in an amount which will differ according to the time of treatment. The function 35 of the protective agent is to protect the silk fiber, or other material, from any possible loss in tensile strength or elasticity and also to remove any tendency of the fiber to become harsh to the touch. As has been said, 40 for a one minute treatment the amount should be about 2 1/2% of the volume of the two other ingredients. For a five minute treatment 5% of glycerine is satisfactory. Good results have been obtained using as 45 high as 15% glycerine.

50 The strength of the formic acid may vary from about 80 to 95%. In the solution above given, 85% formic acid is specified as I have found that this gives very satisfactory results and is easily obtainable on the market. Acid of greater than 95% concentration is very expensive and difficult to obtain. While acids of somewhat less than 80% concentration might give fair results, particularly if 55 the temperature of the solution is raised, best results are obtained within the range given. The strength of the sulphuric acid may also be varied, but for the conditions of treatment above specified, about 95% is believed to be 60 the best. Again, the proportions of the formic acid and sulphuric acid may be changed somewhat without losing the effectiveness of the treatment, but in general there should be about 94 to 99.5 percent 65 formic acid and about .5 to 6 percent sul-

phuric acid. I have secured reasonably satisfactory results with as low as .1% sulphuric acid, but in order to do so I used formic acid of 100% concentration, and this is so expensive as to be prohibitive at the present 70 time.

The actual effect of my treatment on the fibers is, in my opinion, the drawing up or contracting or shrinking of the individual strands and particularly the projecting ends 75 of the fibers that make up those strands. The surface condition of the silk is quite materially changed. It is smoother and firmer, there being little if any fuzz thereon. In the knitted stocking the treatment seems to 80 act on the threads so as to equalize the tension thereon, and if the stocking contains sleazy knitting my treatment removes its characteristic irregular appearance. The smoothness of the treated fibers reduces in 85 large measure the tendency towards picking, and the contraction of the strands and absence of the fuzz gives the stocking a thinner, more sheer appearance.

90 The process of my invention when properly applied should result in no weakening of the fiber and no lessening of its elasticity nor that of the stockings as a whole. In fact, it has been my experience with silk and cotton that the tensile strength and elasticity of the 95 fibers have actually increased as a result of my treatment.

95 From the foregoing it will be seen that my invention is applicable not only to silk stockings but to silk, cotton and other textile materials in any of their many uses. And it will be further understood that substantial variations may be made in the solution and treatment herein described without departing from the spirit and scope of my invention. 105

100 What I claim is:

1. For the treatment of silk, a solution containing formic acid and sulphuric acid, the sulphuric acid content not exceeding 10% by volume of the other ingredients. 110

2. For the treatment of silk, a solution which comprises not less than nine parts formic acid, not more than one part sulphuric acid, and a protective agent.

3. For the treatment of silk, a solution containing formic acid of not less than 80% concentration and sulphuric acid, the formic acid content being not less than 75% by volume of the entire solution. 115

4. For the treatment of silk, a solution containing formic acid of not less than 80% concentration, a protective agent such as glycerine, and concentrated sulphuric acid, the sulphuric acid content not exceeding 10% and the protective agent not exceeding 20% by volume of the entire solution. 120

5. For the treatment of silk, a solution which contains concentrated formic acid, and concentrated sulphuric acid in the proportion 130

of between 98 to 2 and 99.5 to .5, respectively, and glycerine.

6. For the treatment of silk, a solution which comprises about 96½% of 85% formic acid, about 1% of about 95% sulphuric acid, and glycerine in the amount of about 2½% of the volume of the other ingredients.

7. The method of treating silk which consists in subjecting it to the action of a solution containing formic acid and sulphuric acid, and then removing the acid.

8. The method of treating silk which consists in subjecting it to the action of a solution containing concentrated formic acid, concentrated sulphuric acid and a protective agent and then washing the material in an alkaline bath.

9. The method of treating silk which consists in subjecting it for about one minute to the action of a solution containing not less than nine parts of 80 to 100% formic acid, not more than one part of concentrated sulphuric acid, and glycerine in the amount of about 2½% of the volume of the two other ingredients, and then washing the material in an ammonia bath.

10. The method of treating silk which consists in subjecting it for about one minute to the action of a solution containing about 99% of 85% formic acid, about 1% of 95% sulphuric acid, and glycerine in the amount of about 2½% of the volume of the other ingredients, then washing the material for about fifteen minutes in a bath containing 3 to 5 per cent by weight ammonia, and then washing it in water.

11. For the treatment of silk, a solution containing a lower monobasic organic acid and sulphuric acid, the sulphuric acid content not exceeding 10% of the volume of the solution.

CLEO H. KIDWELL.